

Dec. 3, 1968

W. R. KELLY ET AL  
CHROMIZING COMPOSITIONS AND METHODS AND CONTINUOUS PRODUCTION  
OF CHROMIUM HALIDES FOR CHROMIZING

3,414,428

Filed Oct. 20, 1964

2 Sheets-Sheet 1



INVENTORS:  
WALTER R. KELLY  
WILLIAM B. LAUDER  
BY

*Richard E. Vila*

ATTORNEY

Dec. 3, 1968

W. R. KELLY ET AL

3,414,428

CHROMIZING COMPOSITIONS AND METHODS AND CONTINUOUS PRODUCTION  
OF CHROMIUM HALIDES FOR CHROMIZING

Filed Oct. 20, 1964

2 Sheets-Sheet 2



INVENTORS:  
WALTER R. KELLY  
WILLIAM B. LAUDER  
BY

*Richard E. Vila*  
ATTORNEY

3,414,428

CHROMIZING COMPOSITIONS AND METHODS  
AND CONTINUOUS PRODUCTION OF CHRO-  
MIUM HALIDES FOR CHROMIZINGWalter R. Kelly, Geddes, and William B. Lauder, Syra-  
cuse, N.Y., assignors to Allied Chemical Corporation,  
New York, N.Y., a corporation of New YorkFiled Oct. 20, 1964, Ser. No. 405,084  
13 Claims. (Cl. 117—66)

## ABSTRACT OF THE DISCLOSURE

This invention relates to compositions and methods for chromizing of ferrous metal and to the continuous production of anhydrous chromous chloride and chromous bromide; compositions for chromizing comprise a compacted solid intimate mixture of a chromic halide and an activating metal selected from the group consisting of aluminum, zinc, chromium, iron, nickel, magnesium and mixtures thereof.

Chromizing is generally recognized as a low cost method of treating iron and steel to improve the quality of the surface thereof, particularly with respect to oxidation resistance. As distinguished from chrome plating, chromizing methods effect a deposition of chromium metal principally by chemical interchange reaction between a chromium bearing compound and the ferrous metal surface to deposit chromium metal which diffuses into the crystal structure of the ferrous metal and alloys therewith. Thus, chromizing methods are commonly designated as diffusion deposition processes. Pack chromizing techniques are those in which the chromizing composition or mass generating the chromium bearing compound is maintained in contact with the ferrous metal work piece. Usually, the work piece is actually packed in the chromizing composition. Gas phase chromizing processes are those in which the chromizing composition is maintained out of direct contact with the work piece. Fused salt-bath methods have also been proposed.

A known chromizing vehicle is the chromous halide, for example, chromous chloride which deposits chromium metal at the ferrous metal surface according to the reaction:



In diffusion deposition processes of this type it is conventional to introduce controlled amounts of hydrogen gas to expedite deposition of chromium by direct reduction of the chromous halide as illustrated by the reaction:



While the chromous chloride has been used in chromizing, the highly hydroscopic nature of the material has complicated its efficient application. As the chromous chloride should be anhydrous for use in chromizing it has been necessary to generate the chromous chloride in situ to stabilize the material. Further, continuous large-scale production of the anhydrous material has not been practical. Methods developed for these purposes have been relatively complex and have generally introduced other problems which have penalized the chromizing operation. This one factor alone has represented a major obstacle which heretofore has not been effectively overcome in the application of chromous chloride in the chromizing of ferrous metal.

A well-known method developed by Becker, Daeves, and Steinburg (B.D.S. system) is illustrative of the pack or semi-gaseous chromizing process based on chromous chloride. In this method a retort is filled with a mixture

of ceramic lumps and a source of chromium such as ferrochrome and heated to about 1000° C. for 5–10 hours in a circulating stream of HCl gas to convert the chromium to chromous chloride which is held in stabilized form in the pores of the ceramic material. With the chromous chloride impregnated ceramic mass as a convenient source of chromous chloride the ferrous metal work piece is then packed in the ceramic mass and heated to 1000° C. for 5–10 hours to effect deposition of chromium by the above-mentioned interchange reaction. Hydrogen gas is used to deposit chromium directly by the reduction reaction of Equation 2 above. The ceramic chromizing mass in this process may be regenerated for reuse by treatment with HCl gas until the source of chromium has been exhausted. The process results in a satisfactory .004" thick chromium case in about 6–7 hours at the chromizing temperature. While chromium chloride may be effectively handled in this manner, methods of this type essentially involve a two-stage operation requiring considerable processing time and equipment. Such methods also have the particular disadvantage of involving large amounts of the highly corrosive HCl gas which seriously effects the processing equipment which must be frequently replaced.

Gas phase chromizing as illustrated by the method of Hoar and Croom, J. of Iron & Steel Institute, October 1951, involves generating chromous chloride gas by reduction of chromic chloride with hydrogen in a first chamber at 1000° C. and then conducting the chromous chloride vapor with an inert carrier gas over the ferrous metal work piece in a second chamber. Such gas phase methods generally introduce a variety of problems due to the presence of corrosive materials and uneven concentration of the chromous chloride vapors in the vicinity of the base metal. One cause of the corrosion problem in such processes is again the large amounts of HCl gas liberated in the generation of the chromous chloride. Further, a similar action is also caused by the chromic chloride itself which dissociates during the reaction releasing highly corrosive chlorine gas according to the equation:



The ability of the chromic halide to undergo independent dissociation is a deleterious factor in chromizing procedures utilizing such starting material. The free halogen gas liberated thereby is an undesirable diluent in the system which is available to interfere with the chromium deposition reactions and affect the quality of the chromized product. This is supported by efforts to use the chromic chloride as the chromizing vehicle. Results in such cases show not only corrosion of processing equipment but similar attack on the surface of the work piece which is generally severely pitted and of unacceptable quality. Pack and fused salt-bath methods based on in situ generation of chromous chloride from chromic chloride are subject to the same disadvantages.

Attempts to eliminate the problems incident to the use of chromous chloride as the chromizing vehicle have resulted primarily in the development of complex methods requiring highly specific chromizing compositions. A method developed by Diffusion Alloys Ltd. (D.A.L. system) employs a composition consisting of metallic chromium, an inert diluent such as kaolin or chromium oxide, and a solid transfer agent such as ammonium iodide. When the base metal is heated in the presence of the D.A.L. composition, the transfer agent volatilizes expelling undesirable air from the pack and forming chromous iodide from chromium through a complex series of reactions, the chromous iodide then reacting with the ferrous metal and hydrogen to deposit the chromium alloy. Other systems more recently proposed involve the use of compositions containing ammonium bifluorides which may be ap-

plied in liquid form and dried to coat the work piece prior to heating to the chromizing temperature.

It will be evident from the foregoing that several approaches to the chromizing of iron and steel articles have been suggested. However, in the past, chromizing has not been widely utilized and several applications await the development of more efficient methods. While chromous chloride appears to be a highly effective chromizing vehicle the several disadvantages involved in the provision and utilization of this material have been major obstacles to the development of this general type of chromizing procedure.

An object of the present invention is to provide new and improved compositions and methods for chromizing of iron and steel. Another object is to provide new and improved chromizing procedures utilizing chromous halides as the principal chromizing vehicle. Another object is to provide new and improved chromizing compositions and methods utilizing a chromic halide as the source of the chromous halide chromizing vehicle. A further object is to provide new and efficient chromizing techniques in which the chromous halide chromizing vehicle may be generated under substantially non-corrosive conditions. Another object is to provide new and improved chromizing methods in which the chromous halide chromizing vehicle is effectively and efficiently generated from the corresponding chromic halide without deleterious independent dissociation of the chromic halide. Another object is to provide compositions and methods for chromizing in which high purity chromous chloride may be produced in situ as the chromizing vehicle. A further object is to provide a continuous process for chromizing of ferrous metal such as steel strip, wire, and the like. A still further object is to provide a continuous process for production of anhydrous chromous halides for use in chromizing.

Other objects and advantages will be apparent from the following description of the invention.

In accordance with the invention it has been found that metal may be diffusion coated by compositions comprising an intimate mixture of an anhydrous chromic halide selected from the group of chromic chloride, chromic bromide and chromic fluoride and at least about the stoichiometric amount required to convert said chromic halide to the corresponding chromous halide but less than about that amount which would theoretically convert the chromic halide to chromium metal of an activating metal, preferably aluminum, zinc, chromium, or mixture thereof. It has also been unexpectedly found that markedly improved and exceptionally excellent chromizing is obtained by employing the compositions containing the activating metal in an amount of at least about 60% in molar excess of the stoichiometric amount to form the chromous halide, preferably between about 60-130% in excess. Improved results are also achieved by compacting the chromic halide-activating metal compositions to a cake density of at least about 30 pounds per cubic foot, preferably about 60-90 pounds per cubic foot, and particularly when the composition is employed in the form of compacted particles. By employing the chromizing compositions in intimate compacted admixture it has been found that the deleterious dissociation of the chromic halide is suppressed resulting in improved chromizing and appearance of the product. The work piece is left in clean bright condition and ready for immediate use with slight rinsing required if a non-volatile halide is present.

Iron and steel articles are diffusion coated in accordance with the invention by reactively heating the chromizing composition in an oxygen-free and moisture-free atmosphere at a temperature above about 470° C. to convert the chromic halide to a lower valence-state chromium halide reaction product or chromizing mass and contacting the ferrous metal with the resulting chromium halide reaction product at a temperature within the range of about 820° C. to 1300° C., preferably 1000° C.

to 1300° C., for a time sufficient to diffusion coat the desired amount of chromium on the ferrous metal, said diffusion coating being carried out while maintaining an oxygen and moisture-free atmosphere. An inert gas stream such as argon is generally employed to maintain an inert atmosphere and facilitate the deposition of chromium by interchange reaction at the surface of the ferrous metal. If desired, controlled amount of hydrogen may be employed to expedite chromium deposition by direct reduction of the chromium halide vapors in the system. The compositions containing the chromic halide and an activating metal may, in addition to packed chromizing procedures, be adapted to obtain improved chromizing in gas phase and fused salt-bath techniques and also are well suited for continuous chromizing and the continuous production of high purity chromous halides. Improved chromizing rates over conventional methods for both pack and vapor phase chromizing have also been found. In pack chromizing, 1-2 hours suffice to produce a satisfactory case of .001-.002 inch thickness while cases of the same thickness and quality have been applied to only 10-40 minutes when gas phase chromizing techniques are employed. Articles having a high oxidation resistance approaching 410 stainless steel may be obtained with cases of only about .001" in thickness. Complex work pieces having recessed surfaces are also readily coated with uniform chromium cases.

Proportions in which the chromic halide and activating metals are admixed may be varied depending on the type of chromizing procedure and particular metal employed. Generally, the lower limit for the activating metal is about the stoichiometric amount required to convert the chromic halide present to be corresponding chromous halide. Lesser amounts do not effectively suppress dissociation of the chromic halide and do not result in uniform chromizing of the ferrous metal. The upper limit is less than the amount of metal which would theoretically convert the chromic halide present to chromium metal and preferably no more than about 67% of that amount. In cases where trivalent aluminum metal is employed, mol ratios of the chromic halide to aluminum would be 3:1 or lower. For the other indicated finely divided metals such as zinc, iron, chromium, etc. the mol ratio of chromic halide to metal would be 2:1 or lower. It has been found unexpectedly that markedly improved and exceptionally excellent results are obtained by employing compositions containing an excess over the stoichiometric amount of metal required to form the chromous di-halide, desirably a molar excess between about 60% to 130%. Preferred ratios of chromic halide to aluminum metal are therefore within the range of about 3:1.6 to 3:2.3 and most desirably a ratio of about 3:2. For other metals (divalent) with exception of chromium preferred ratios are within the range of about 2:1.6 to 1:1.3, and most desirably a ratio of about 1:1. When employing chromium metal the actual molar excess may range up to about 330% or about 30% in excess of the amount which would form the monohalide CrCl. In general, use of a molar excess of the activating metal has been found to have the particular advantage of requiring shorter processing times and little or no hydrogen gas to obtain excellent and optimum chromium decomposition. Thus, chromium cases having high total chromium deposit and high oxidation resistance approximating 410 stainless steel are produced within short chromizing periods whether or not hydrogen is employed. (In such preferred embodiments very minor amounts of hydrogen may be useful as scavenger for free or dissociated chlorine in the system.) The finished product is also characterized by improved brightness qualities. While it is not certain why a stoichiometric excess of metal is advantageous, it is believed that the chromic halide-activating metal reaction result in a product containing monohalide, such as CrCl, or other equivalent product (such as a vaporous mixture of CrCl<sub>2</sub> and chromium) which is a highly effective vehicle in the chromium deposi-

tion reaction. In practice of the invention, it is, therefore, contemplated that the lower valence-state chromium halide reaction product be or contain chromium halide in which the chromium has a valence of two or below. Therefore, when hereinafter reference is made to chromous halides or chromium halide reaction product, mixtures containing lower halides of chromium are included. In any event, the invention, particularly in its preferred aspects, makes possible chromizing in a system consisting essentially, or even solely, of the chromic halide and activating metal as the solid reactants. By employing a stoichiometric excess of activating metal, it has also been found that chromium cases of only a minimum .001 inch thickness have excellent oxidation resistance.

Compaction of the chromic halide-activating metal compositions is a feature of the invention and has been found to give excellent results where the uncompacted composition was less than satisfactory, particularly in packed chromizing procedures. Very bright and quality finishes are obtained by compaction indicating that compaction results in an exacting control of the deleterious properties of the chromic halide starting material. Further advantages are realized by employing the compacted composition in the form of compacted particles and particularly in pack chromizing procedures when complex articles are to be coated. Improved chromizing rates are also realized by compacting the composition. Compaction of the chromizing compositions may be accomplished under pressure by known methods. Compaction pressures of about 750-2500 p.s.i.g. are suitably employed for this purpose. Apparatus may be any suitable conventional device such as an hydraulic press or pellet maker. The activating metal is preferably finely divided with a size of less than about 100 Tyler standard mesh, and most desirably is employed in powdered form with a mesh size within the range of about 100 to 325 Tyler standard mesh. The anhydrous chromic halide employed has a mesh size preferably less than about 100 Tyler standard mesh, and desirably within the range of about 100 to 325 standard mesh. The chromic halide-activating metal composition before compaction has typically a fine particle size and a bulk density of about 3-12 pounds per cubic foot. The compacted mass should have a cake density of at least about 30 pounds per cubic foot and improved results are obtained with cake densities of up to 90 pounds per cubic foot. Higher densities may be employed although a cake density of about 120 pounds per cubic foot is about the practical upper limit above which no substantial additional advantages are obtained. The compacted particles may be readily formed by breaking up the compacted composition and screening the mass. Particle size may be varied over a fairly wide range. Suitable results are obtained when compacted particles having a Tyler standard mesh size within the range of about 100 to 8, preferably within the range of 100 to 20 Tyler standard mesh. Compaction and the retention of particle shape is enhanced by the platelet character of the chromic halide. In addition to improved chromizing, compaction enables easy handling and storage and also improves flow quality to give a material eminently suited as a feed for gas phase and fused salt-bath chromizing processes.

The indicated finely divided activating metals may be admixed in the designated proportions depending on preferred conditions and results desired during the chromizing operation. By-product activating metal halides formed during the reaction do not interfere with the chromizing reaction and do not represent a corrosion factor as is the case when chromic chloride and hydrogen are employed. In all forms of the invention, a preferred chromizing composition contains chromic chloride and finely divided aluminum which react to produce the chromizing reaction product and by-product aluminum chloride which separates from the reaction mixture. Such composition enables the generation in situ of a high purity chromizing mass and the production of high quality chromium cases.

When such compositions are employed, the generation of the chromizing mass and the release of by-product aluminum chloride are essentially completed at about 500° C. or well below chromizing temperatures as evidenced by change in color of the composition from the violet attributed to chromic chloride to a gray color and by cessation of evolution of the white vapors of aluminum chloride at about this temperature. A high purity chromizing mass such as obtained with aluminum may also be produced with zinc, the only observable difference being that evolution of by-product zinc chloride vapor occurs at a somewhat higher temperature of about 730-750° C. Similarly, compositions composed of chromic halide and chromium metal yield a high purity chromizing mass and also have the particular advantage of involving no by-product formation.

In practice of the invention both the reaction generating the chromium halide product and the chromizing reaction may be carried out in a single uninterrupted operation. Thus, in pack chromizing procedures the work piece may be filled with or may be surrounded or placed in contact with the chromizing composition and the charge heated to the chromizing temperature above about 820° C., preferably a temperature within the range of about 1000° C. to 1300° C. During the heating operation the chromic halide is readily converted at temperatures of about 500° C. to the lower-valence chromium halide reaction product containing the corresponding chromous halide. As the chromizing temperatures are reached the chromium halide reaction product chromizes the work piece by surface diffusion and interchange replacement of the ferrous metal. Heating time to the chromizing temperature is not particularly important and is generally carried out over the course of about 3 to 4 hours. Variable amounts of hydrogen gas may be employed to deposit chromium directly by reduction of the chromium halide reaction product and to increase the amount of chromium deposited and the chromium deposition rate. Generally, hydrogen is most beneficial when the activating metal is used in amounts which are stoichiometric, e.g. chromic halide to aluminum ratios of about 3:1. In a preferred pack chromizing procedure, the chromizing composition is made up of compact particles of an intimate mixture of chromic chloride and powdered aluminum metal in a mol ratio within the range of about 3:1.6 to 3:2.3. The particulate mass has a size preferably within the range from about 100 to 20 standard mesh. The pack is then heated and at temperatures of about 500° C., the chromic chloride is converted forming by-product aluminum chloride which vaporizes from the vicinity of the work piece leaving the work piece surrounded by high purity chromium chloride reaction product. Pack chromizing temperatures are preferably within the range of 1000-1200° C. with excellent results obtained after about 2 hours at the chromizing temperature. Longer chromizing periods, as much as 4 to 6 hours, may be employed where heavy duty chromium cases are desired. Generally, pack chromizing procedures may be conveniently carried out at atmospheric pressure although a slight positive pressure may be maintained within the chromizing apparatus to prevent the introduction of air. The reaction is carried out under oxygen-free and moisture-free conditions to prevent corrosive attack on the work piece. An inert gas such as argon is generally circulated through the reaction mass for this purpose and to facilitate contact of the reactive chromium halide with the surface of the work piece. Other inert gases such as helium may also be employed.

In another embodiment of the invention a gas phase or semi-gas phase chromizing operation is conducted by suspending a work piece in the upper portion of a suitable reactor with the chromizing composition placed in a lower portion and in the vicinity of the work piece but out of contact therewith. Generally, a distance of about 1/4 to 4 inches, preferably about 2 inches, separates the work piece from the chromizing composition. In this manner

the chromizing may be carried out without complete vaporization of the chromizing mass as the partial pressure vapors of the chromizing mass contact the work piece and effect the desired chromizing action. By such procedure gas phase chromizing may be carried out at a preferred temperature within the range of about 1100° C. to 1200° C. It will be understood, however, that in gas phase procedures the composition may be placed at any suitable distance from the work piece and operating conditions maintained to completely vaporize the generated chromizing mass. In gas phase operation iron, nickel and magnesium may also be employed as activating metals. Generally, the preferred gas phase chromizing compositions are also compacted particles of chromic chloride and powdered aluminum metal in the mol ratio of about 3:1.6 to 3:2.3, most desirably about 3:2.

In the semi-gas phase operations the composition is heated to generate the lower valence chromium halide chromizing mass and by-product aluminum chloride which is vaporized from the mixture. The aluminum chloride by-product may be released from the system and recovered, but this procedure is not necessary as the aluminum chloride does not interfere with the chromizing reaction. The chromizing mass thus formed is then heated to temperatures preferably within the range of 1100° C. to 1200° C. and vapors from the resulting molten chromizing mass contact the ferrous metal work piece and effect the chromizing action. A circulating stream of an inert gas such as argon is generally employed to maintain air-free and moisture-free conditions and facilitate contact of the chromium halide with the work piece. Gas phase chromizing procedures carried out in this manner will form uniform chromium cases of .001"- .002" thickness having high oxidation resistance in as little as about 10 to 40 minutes. The chromizing time may be extended to periods as long as 1.6 to 4.9 hours to produce work pieces having .003" to .005" cases, respectively. Generally, a slight positive pressure or atmospheric pressure is employed in gas phase operations as desired, although reduced pressures may be used to advantage to maintain gas phase conditions, particularly with the less volatile chromous fluoride reaction product.

Another feature of the invention is continuous operation adapted for either continuous production of chromous halides or continuous chromizing of ferrous metal articles such as strip, wire, and the like.

The embodiments of the invention adapted for continuous operation will be further described in detail with reference to the accompanying drawings, in which:

FIG. 1 shows in cross-sectional elevation a preferred form of apparatus for continuous chromizing of ferrous metal such as strip, wire, and the like.

FIG. 2 shows in cross-section elevation a preferred form of apparatus for continuous production of anhydrous chromous halides.

Referring to the drawings, FIG. 1 illustrates a preferred form of apparatus in which the compositions of the invention may be employed in continuous chromizing. As shown in FIG. 1, apparatus for continuous chromizing generally includes a chromium halide generator 10 and chromizing chamber 11. In carrying out this embodiment of the invention, there is continuously fed to the chromium halide generator 10 a composition comprising an intimate mixture, preferably compacted and desirably in the form of compacted particles, of anhydrous chromic halide selected from the group consisting of chromic chloride and chromic bromide and at least about the stoichiometric amount required to convert said chromic halide to the corresponding chromous halide but less than about that amount which would theoretically convert the chromic halide to chromium metal, preferably a stoichiometric excess of a finely divided activating metal selected from the group consisting of aluminum, zinc, chromium, and mixtures thereof, preferably alumini-

num. The chromium halide generator 10 is maintained under oxygen and moisture-free conditions and at a temperature within the range of about 820° C. to 1300° C., preferably 900° C. to 1000° C., to convert the chromic halide-activating metal feed composition to the chromium halide reaction product which is then withdrawn in a molten form from generator 10 and introduced into chromizing chamber 11. Chromizing chamber 11 is maintained under air-free and moisture-free conditions, usually with the aid of a circulating stream of an indifferent gas, and at a chromizing temperature within the range of about 820° C. to 1300° C., preferably a temperature within the range of about 1100° C. to 1200° C. The ferrous metal to be chromized is continuously introduced into the chromizing chamber and passed therethrough in the vicinity of the molten chromium halide reaction product to cause the chromium halide product, preferably in the form of vapors of said product, to contact the surface of the ferrous metal and effect the chromizing action.

As shown in FIG. 1, the chromium halide generator assembly includes a hopper 12 in which the feed composition is placed. Hopper 12 is preferably covered and may be gas-pressurized, if desired. The composition may also be maintained under inert conditions by the introduction of an indifferent gas through line 13. The chromizing composition is withdrawn from hopper 12 and transferred by feed screw conveyor 14 or other suitable type feeder through line 16 into a generally vertical reaction zone 17. The composition in line 16 is maintained under an inert atmosphere during transfer to reaction zone 17 by an indifferent gas supplied through inlet line 18 and discharged through outlet line 19. Reaction zone 17 is equipped with an overflow standpipe 21 connected to chromizing chamber 11 and overflow stand pipe 23 which has plurality of openings 22 at the bottom to permit the molten chromium halide product to flow to the top of the overflow stand pipe. Inlet tube 24 terminates above the level of the reactants in reaction zone 17 and introduces an indifferent gas to maintain an otherwise inert atmosphere in the reaction zone and facilitate removal of by-product vapors formed during the chromium halide generating reaction. Tap line 25 serves as convenient means for withdrawing samples of the chromium halide reaction product. Reaction zone 17 is externally heated by suitable means (not shown) and at least the lower portion of the reaction zone continuously maintained at a temperature within the range of about 820° C. to 1300° C., preferably a temperature of about 900° C. to 1000° C., or sufficient to maintain adequate fluidity of the molten chromium halide reaction product in the lower portion of reaction zone 17. Upper zone temperatures are mostly a matter of maintaining removable by-product in vapor form and, if desired, may be as low as 200-300° C. in cases where by-product  $AlCl_3$  is produced. The rate of feed of the composition to reaction zone 17 is governed by the chromium halide reaction product requirements in the chromizing chamber. Under the indicated temperature conditions, the feed composition is rapidly converted in the lower portion of reaction zone 17 to a molten chromium halide reaction product or chromizing mass. Volatile by-product activating metal halides formed during the generating reaction are removed from the reaction zone through sublimate outlet 26 with the aid of the indifferent gas introduced through inlet tube 24. Thus, in a preferred embodiment in which aluminum is used in the make-up of the feed composition, the by-product aluminum chloride vapors exit reaction zone 17 through outlet 26 and pass through sublimate duct 27 to sublimate condenser 28. Solid aluminum chloride by-product may be withdrawn, as desired, from sublimate condenser 28 through condenser outlet 29 and collected in a sublimate receiver (not shown). The by-product recovery assembly is equipped with a manually operated helical ream-out 30 to remove any prematurely con-

densed material which might block inlet 26 and sub-limate duct 27.

From reaction zone 17, the molten chromium halide reaction product is transferred by gravity through standpipe 21 to chromizing chamber 11. The chromium halide product may be transferred dripwise or as a continuous stream depending on the requirements in the chromizing chamber. Standpipe 21 is also equipped with an inlet tube 31 for introduction of an indifferent gas to maintain the molten chromium halide product under inert conditions during transfer to the chromizing chamber. The chromium halide reaction product entering the chamber becomes a part of the chromizing mass 32 which is disposed on the bottom of the chamber. Chromizing mass 32 is preferably distributed over the full length of the chamber bottom to permit maximum chromizing time within the chamber. The ferrous metal being chromized, for instance a steel strip 33, is continuously drawn through the chromizing chamber 11. Although the ferrous metal may be immersed in chromizing mass 32 this procedure is less desirable and the ferrous metal 33 is preferably maintained throughout passage through the chamber in sufficient proximity to the chromizing mass to permit vapors of the mass to contact and surround the strip and thereby effect the chromizing action. Distance between the chromizing mass and the material being chromized may be varied depending upon conditions maintained in the chromizing chamber. Generally, a distance of about  $\frac{1}{4}$  to 4", preferably about 2", separates the material being chromized from the molten chromizing mass. Strip 33 is continuously withdrawn from a pay-out spool 34 which is enclosed in a housing 36. Walls 37 and 38 separate housing 36 from the chromizing chamber 11. Strip 33 is fed through a slit 39 which is preferably sufficiently air tight to prevent passage of vaporous material from the chromizing chamber to the housing and to prevent air from entering the chromizing chamber. Generally, an indifferent gas is introduced into housing 36 through inlet 41 to ensure oxygen and moisture-free conditions in the system. Chromizing chamber 11 is externally heated by suitable means (not shown) to continuously maintain the chromizing mass at a temperature within the range of about 820° C. to 1300° C., preferably a temperature within the range of 1000° C. to 1200° C. to effect the chromizing action on the metal strip 33. Chromizing chamber 11 is maintained throughout the operation under oxygen-free and moisture-free conditions to prevent undesirable side reactions and corrosive attack at the surface of the work piece. This is suitably accomplished by circulating a stream of an indifferent gas through chromizing chamber 11. For this purpose chamber 11 is fitted with an inlet tube 42 for introduction of indifferent gas and an outlet tube 43 through which the indifferent gas exits the chamber after circulation therein. The use of a circulating stream of an indifferent gas in this manner also serves to facilitate removal of any by-product vapors from the surface of the work piece and chamber thereby promoting optimum operating conditions. Hydrogen gas may also be employed in continuous chromizing to deposit chromium by direct reduction of the chromium halide product. For this purpose the hydrogen gas is most conveniently introduced along with the indifferent gas entering inlet tube 42 with by-product vapors being rapidly removed from the vicinity of the work piece and chromizing chamber along with the gas stream exiting outlet tube 43. Variable amounts of hydrogen gas may be employed depending on operating conditions and chromium deposit desired. However, in continuous as well as the previously discussed batch chromizing procedures, little or no hydrogen gas is necessary to facilitate chromium deposition when the indicated preferred ratios are used in the make-up of the feed composition.

The rate of passage or exposure time during which the work piece is subjected to vapors of the chromizing

mass may be varied over a fairly wide range, and may be as little as 2 minutes to as much as 2 hours. In continuous operation, case thicknesses of the order of .0005 to .005 inch and total chromium deposit averaging 15-25% chromium are obtainable. Exposure time during passage of strip 33 through chromizing chamber 11 depends on several factors and varies primarily with the chromizing temperature, the amount of chromium deposit and thickness of the case desired during the operation, and length of the chromizing chamber. Length of the chromizing chamber 11 is mostly a matter of convenience and economy and is typically within the range of about 3 to 15 feet, preferably about 15 feet in length. The higher chromizing temperatures result in higher chromium deposition rates and permit higher rates of passage of the work piece through the chromizing chamber. Lower rates are required in situations where it is desired to obtain thick cases having high total chromium deposit. Under preferred operation conditions, case thickness averages .001 to .002 and having good oxidation resistance may be obtained with exposure times of about 11 to 43 minutes. Chromized steel strip and wire of this quality are eminently suited for use in several applications including mufflers, trim, and wire.

The chromized strip is continuously withdrawn from the chromizing chamber for recovery through a slit 44 which is also designed to be sufficiently air tight to prevent passage of air into the chromizing chamber. The chromized strip is then wound on take-up spool 46 located in housing 47. If desired, the strip may be quenched or cooled by other suitable means after removal from the chamber and prior to recovery. Take-up spool 46 is rotated at the desired rate by a variable speed motor and gear-transmission (not shown) which are connected to the take-up spool shaft 48. An indifferent gas is also introduced into housing 47 through inlet 49 to ensure oxygen-free and moisture-free conditions. In operation, chromizing is generally carried out at atmospheric pressure although a slight positive pressure may be employed to further prevent air from entering the chromizing chamber.

Chromium halide generator 10 and chromizing chamber 11 are generally constructed of a suitable corrosion-resistant material, preferably stainless steel. Other materials which can be used include Inconel and chromized steel. By employing the compositions of the invention comprising an intimate mixture of anhydrous chromic halide and finely divided activating metal, preferably in compacted form, the deleterious corrosion-inducing characteristics of the chromic halide which under chromizing conditions attacks materials such as stainless steel are effectively suppressed. Thus, the apparatus remains corrosion free over an extended period of operation and has a long useful life. In continuous operation the indifferent gas employed to maintain inert conditions is preferably argon although other gases, such as helium, which are inert under the operating conditions may also be used.

Another feature of the invention includes the use of the chromic halide-finely divided activating metal compositions in the continuous production of high purity anhydrous chromous halides suitable for use in chromizing. Apparatus for this purpose is shown in FIG. 2 and is substantially the same as apparatus shown and described with reference to FIG. 1 except that the chromizing chamber and accessories are substituted by suitable means for recovery and for cooling the chromous halide product. In FIG. 2, part numbers designate the same parts shown by like part numbers in FIG. 1.

Referring to FIG. 2, method for continuous production of anhydrous chromous halides involves conversion of chromic halide-finely divided activating metal feed composition in generator 10 by substantially the same procedure employed in continuous chromizing operations.

The feed composition for continuous production of chromous halides is more closely proportioned than that

for continuous chromizing procedures and comprises an intimate mixture, desirably compacted and preferably in the form of compacted particles, of anhydrous chromic chloride or chromic bromide and about the stoichiometric amount required to convert said chromic halide to the corresponding chromous halide of an activating metal selected from the group of aluminum, chromium, and zinc. A preferred composition for production of high purity anhydrous chromous halide comprises compacted particles of the chromic halide and powdered aluminum metal in the mol ratio of about 3 to 1. In this embodiment of the invention, the feed composition is continuously withdrawn from the storage hopper 12 and introduced through line 16 into generator 10 where it passes by gravity to the lower portion of reaction zone 17. Conversion to the anhydrous chromous halide product takes place generally at a temperature of about 470° C. to 500° C. and at least the lower portion of reaction zone 17 is maintained at a temperature within the range of about 820° C. to 1300° C., preferably a temperature of about 900° C. to 1000° C., to assure adequate fluidity of the product. Reaction zone 17 is continuously maintained under oxygen and moisture-free conditions by introduction of an indifferent gas, preferably argon, through line 24. Depending on feed rate of the composition the molten anhydrous chromous halide product is withdrawn dripwise or in the form of a continuous stream from reaction zone 17 by gravity flow through overflow standpipe 21 which is connected to product recovery receptacle 51 by union nut 52 in such a manner as to prevent oxygen or moisture from entering the receptacle and contacting the product. The molten product flows from the standpipe 21 into a drip tube 53 and descends in free fall through the upper portion of the receptacle including the flanged cap 54 which is secured by bolts and suitable gasket (not shown) to the receiver housing 56. The standpipe 21, drip tube 53 and flanged cap 54 are all preferably heated by suitable means (not shown) to prevent pre-solidification of the product in the upper portion of the recovery receptacle 51. The descending molten chromous halide is deposited on two closely spaced rotating rolls 57 which are driven on shafts 58 connected by suitable means to a motor (not shown) which is located outside the recovery receptacle 51. Rolls 57 are cooled by air or other gas supplied and withdrawn through the shafts 58 which are made hollow for this purpose. The chromous halide is solidified on the cooled rolls and removed therefrom on rotation by scraper knives 59. The solid chromous halide from the rolls descends into the receiving tray 61 which may be removed and replaced as desired through the retrieval door 62. In operation, the recovery receptacle 51 is maintained under air- and moisture-free conditions by an indifferent gas introduced through inlet purge tube 63 and withdrawn through outlet tube 64. To insure inert conditions an indifferent gas is also introduced through inlet tube 31 into the overflow standpipe 21. Substantially 100 percent conversion of the chromic halide to the corresponding anhydrous chromous halide is obtained in the generator under the indicated conditions. The recovered anhydrous chromous halide product may be stored under moisture-free conditions for use in chromizing or other situations where the high purity material is desired.

The following examples illustrate the present invention.

#### Example 1

This test was conducted to show that the chromizing mixture of the invention results in the quantitative formation of the chromous chloride chromizing vehicle, and more particularly that a composition composed of chromic chloride and a stoichiometric amount of powdered aluminum produces quantitatively high purity chromous chloride, M.P. 815-820° C. Compacted particles (cake density 60-90 pf.) of an intimate mixture of CrCl<sub>3</sub> and powdered aluminum in the mol ratio of about 3:1 were placed in

5 a Vycor boat which was inserted in a 1 inch horizontal Vycor tube. The charge was then slowly heated to a temperature of about 1000° C. over a period of about 2 hours while under an argon atmosphere. As the temperature reached the vicinity of 470° C. as measured by a thermocouple, white vapors of AlCl<sub>3</sub> evolved from the reaction mass. The purple color of the particle mass ascribed to CrCl<sub>3</sub> gave way to a gray white powdery residue ascribed to CrCl<sub>2</sub>. At a temperature of about 500° C. the evolution of the white vapors of AlCl<sub>3</sub> ceased and the gray-white powdery residue was observed to have a melting point temperature of about 820° C., demonstrating the formation of chromous chloride in a substantially pure state.

#### Example 2

This test was conducted to show the desirability of compacting the composition in packed chromizing procedures. The chromizing composition was an intimate mixture of anhydrous chromic chloride and powdered aluminum metal in the mol ratio of 3:1. Into a mild steel specimen having closely spaced turns and a total surface area of 125 sq. in. and a stock thickness of only 0.002 inch, was packed as much of this low bulk density composition as physically possible. This amounted to only 25 3 grams. The loaded specimen was placed in an Inconel retort. The retort was closed and heated to 1100° C. and held at this temperature for 2 hours. During the heat cycle a gas stream containing argon plus hydrogen gas was passed through the retort. The average argon gas flow rate was about  $20 \times 10^{-3}$  s.c.f.m. while the limited hydrogen flow rate was about  $6 \times 10^{-3}$  s.c.f.m. The retort was then allowed to cool to ambient temperature and the specimen removed from the retort and evaluated as to appearance and oxidation resistance. The general appearance of the piece was good but the oxidation resistance of the chromized specimen for 6 hrs. at 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910

.0006 inch thick, and a total chromium deposition of about 11% of the weight of the specimen. Oxidation resistance test showed 170 mg./dm.<sup>2</sup> weight gain in 6 hours at 1200° F.

*Example 4*

Example 4 was conducted the same as Example 3 except that the chromizing composition for Example 4 contained chromic chloride and aluminum metal in a mol ratio of 3 to 1.5. It was found that the product had a surface with the bright appearance of chromium metal. Metallographic examination of the surface showed an alloyed chromium case .0006 inch thick and a total chromium deposition of about 12% of the weight of the specimen. Oxidation resistance test showed 80 mg./dm.<sup>2</sup> weight gain in 6 hours at 1200° F.

*Example 5*

Example 5 is presented to show that as the mol ratio of CrCl<sub>3</sub> to Al approaches 3:2, a further marked improvement in chromizing is noted. Hence, Example 5 was conducted the same as Examples 3 and 4 except that the mol ratio of chromic chloride to aluminum metal in the chromizing composition was 3 to 1.76. It was found that the product had a surface with the bright appearance of chromium metal. Metallographic examination of the surface showed an alloyed chromium case .001 inch thick and a total chromium deposition of about 18%. Oxidation resistance test showed 5 mg./dm.<sup>2</sup> weight gained in 6 hours at 1200° F. This compares with an oxidation resistance of about 7 mg./dm.<sup>2</sup> for 410 stainless steel tested under the same conditions. The mild steel stock was only .002" thick to begin with. A case of .001" means that, for all practical purposes, the chromized piece had become all case.

*Example 6*

For Example 6 the chromizing composition was prepared by intimately mixing 2.4 parts by weight of anhydrous chromic chloride and 1 part by weight of powdered zinc metal. The mol ratio of chromic chloride to zinc metal in the resulting mixture composition was 1:1. The mixture was compacted under a pressure of 750 p.s.i.g. in a standard pellet press to a cake density of about 90 pounds per cubic foot and then broken up and classified by screening. Particles in the range of 100 to 20 standard mesh were selected for use. The specimen and procedure employed were the same as Examples 3-5, inclusive. The product had a surface with the bright appearance of chromium metal. Metallographic examination of the surface showed an alloyed chromium case 0.0009 inch thick and a total chromium content of 8%. Oxidation test showed 9 mg./dm.<sup>2</sup> weight gain for 6 hours at 1200° F., or practically as good as 410 stainless steel under the same test conditions.

*Example 7*

Example 7 is a pack-gas phase chromizing procedure conducted in the same two-piece stainless steel retort as used in the preceding examples. The retort had a cylindrical cover section of 5" diameter and an overall height of about 6" with the closed top fitted with 1/4" stainless steel inlet and outlet tubes. The interior of the cover section had a generally bell-shaped configuration. The base section of the retort comprises two stainless steel cylindrical cups with one placed inside the other and separated by -100 mesh aluminum oxide which is employed as a porous seal adapted to maintain a slight positive pressure while allowing effluent gases to escape from the retort. The diameter of the outer cup is about 5 1/2" with a height of about 6" and the diameter of the inner cup is about 4 1/2" with a height of about 5". A small stainless steel U-shaped rack mounted on a generally circular base is positioned on the bottom of the inner cup. Four 2 1/2" x 1" x .0037" specimen strips of

1010 steel were used. The four strips were each pierced by 2 holes at their extremities so that they could be slipped onto the two upright posts of the U-shaped rack. They were separated from each other by 1/2" ceramic blocks. A total of 9 grams of a mixture of chromic chloride and powdered aluminum metal in the mol ratio of 3:2 was placed on the strips. The strips resembled a four-decker sandwich with spaces between, the mixture lying on the top of each strip about 1/4 inch from the steel specimen immediately above. The cover section of the retort was then fitted between the vertical walls of the lower section of the retort and depressed 1/2" into the Al<sub>2</sub>O<sub>3</sub> powder. A ring of 1/2" asbestos rope was then disposed in the annular space between the outer wall of the cover section and the inner surface of the outer wall of the 5 1/2" diameter cup and pressed firmly into the aluminum oxide seal. The retort was fastened tightly together by wire and placed in the furnace in upright position and heated for about 4 hours to 1100° C. The temperature was kept at 1100° C. for 2 hours. A mixture of hydrogen and argon gas was fed to the retort. The rate of flow of argon gas was about  $20 \times 10^{-3}$  s.c.f.m. The rate of flow of hydrogen gas was  $7 \times 10^{-3}$  s.c.f.m. All specimens were found to have a uniform bright deposit of chromium metal. Analysis of the surface showed a case of 0.0009 inch and a total chromium deposit of about 9.05%. Oxidation resistance tests showed only 20 mg./dm.<sup>2</sup> weight gained for 6 hours at 1200° F.

*Example 8*

Example 8 demonstrates the omission of hydrogen and gas phase chromizing with the four 2 1/2" x 1" x .0037" specimen strips of the preceding Example 7 suspended from the horizontal top bar of a T-shaped rack. A total of 9 grams of the CrCl<sub>3</sub>/Al mixture of mol ratio 3:2 was disposed a distance of 1" from the strips. The strips were hung facing each other at even distances. The chromizing mixture was placed at the base of the T-shaped rack. The chromizing retort, argon flow rate, temperatures and time at 1100° C. were the same as in Example 7. All specimens were found to have a uniform bright deposit of chromium metal. Analysis of the surface showed an alloyed chromium case of 0.0009 inch and a total chromium deposit of about 9.97%. Oxidation resistance tests showed only 18 mg./dm.<sup>2</sup> weight gained for 6 hours at 1200° F.

Although certain preferred embodiments of the invention have been disclosed for purpose of illustration, it will be evident that various changes and modifications may be made therein without departing from the scope and spirit of the invention.

We claim:

1. A composition for use in the diffusion coating of ferrous metal with chromium by interchange reaction of a chromium halide and said ferrous metal comprising a solid, compacted intimate mixture of an anhydrous chromic chloride, chromic bromide, and chromic fluoride and at least about the stoichiometric amount up to about 330% molar excess of the amount required to convert said chromium halide to the corresponding chromous halide, but less than that amount which would theoretically form chromium metal from the chromic halide of a finely divided activating metal selected from the group consisting of aluminum, zinc, chromium, iron, nickel, magnesium, and mixtures thereof; said compacted mixture having a cake density of 30 to 120 pounds per cubic foot.
2. The composition of claim 1 in which the activating metal is present in an amount of at least about 60% in excess of the stoichiometric amount.

3. The composition of claim 1 in which the activating metal is present in a molar excess up to about 130%.
4. The composition of claim 1 wherein the mol ratio of chromic halide to activating metal is from about 3:1 to 1:1.3.

## 15

5. The composition of claim 1 in which the activating metal is aluminum.

6. The chromizing composition of claim 1 in which the activating metal is zinc.

7. The chromizing composition of claim 1 in which the activating metal is chromium.

8. The composition of claim 1 wherein the anhydrous chromic halide is chromic chloride.

9. The composition of claim 5 in which the chromic halide is chromic chloride and the mol ratio of chromic chloride to aluminum is within the range of about 3:1.6 to 3:2.3.

10. The composition of claim 1 in which the compacted mixture has a cake density within the range of about 30 to 90 pounds per cubic foot.

11. The chromizing composition of claim 1 in which the intimate compacted mixture is in the form of compacted particles having a Tyler standard mesh size within the range of about 8 to 100.

12. In a method of chromizing ferrous metal which comprises contacting the ferrous metal with a chromium halide chromizing agent in an oxygen-free atmosphere at a temperature within the range of about 820° to 1300° C. for a time sufficient to chromize said ferrous metal, the improvement comprising the use of a solid, compacted, intimate mixture of an anhydrous chromic halide selected from the group consisting of chromic chloride, chromic bromide, and chromic fluoride and at least about the stoichiometric amount up to about 330% molar excess of that amount required to convert said chromic halide to the corresponding chromous halide, but less than that amount which would theoretically form chromium metal from the chromic halide of a finely divided activating metal selected from the group consisting of aluminum, zinc, chromium, iron, nickel, magnesium, and mixtures

5

10

15

20

25

30

35

## 16

thereof, said compacted mixture having a cake density of 30 to 120 pounds per cubic foot.

13. The method of claim 12 wherein the solid, compacted, intimate mixture of the chromic halide and activating metal is fed to a first zone maintained under inert conditions at a temperature within the range of about 820-1300° C. to convert the chromic halide to a molten chromium halide product, withdrawing said molten chromium halide product from said first zone, passing said molten product while maintaining inert conditions to second zone, continuously introducing the ferrous metal into said second zone, maintaining said second zone under inert conditions and at a temperature within the range of about 820 to 1300° C., continuously passing the ferrous metal within said second zone in the vicinity of the molten chromium halide product to cause vapors of said chromium halide to diffuse the surface of said ferrous metal to deposit chromium metal, and continuously withdrawing chromized ferrous metal from said second zone.

## References Cited

## UNITED STATES PATENTS

|           |         |                 |       |             |
|-----------|---------|-----------------|-------|-------------|
| 2,304,463 | 12/1942 | Maier           | ----- | 23—87       |
| 2,762,700 | 9/1956  | Brooks          | ----- | 23—87 X     |
| 2,801,187 | 7/1957  | Galmiche        | ----- | 117—107.2 X |
| 2,887,984 | 5/1959  | Drummond        | ----- | 117—107.1 X |
| 3,021,231 | 2/1962  | Samuel et al.   |       |             |
| 3,152,007 | 10/1964 | Perrin et al.   | ----- | 117—107.2   |
| 3,244,477 | 4/1966  | Nicco et al.    | ----- | 23—87       |
| 3,252,823 | 5/1966  | Jacobson et al. | ---   | 117—107.2 X |

ALFRED L. LEAVITT, Primary Examiner.

A. G. GOLIAN, Assistant Examiner.